# EUROPEAN PATENT SPECIFICATION

(11) **EP 0 677 572 B1**
(45) Date of publication and mention of the grant of the patent: **07.01.1999**
(21) Application number: 95105672.0
(22) Date of filing: 13.04.1995
(51) Int. Cl.: C10M 159/12, C10M 133/52, C10M 177/00

(54) **Detergent-dipersant additive for lubricating oils of internal combustion engines and its preparation process**
Detergensdispergiermittelzusatz für Schmieröle für Verbrennungskraftmaschinen und Verfahren zu dessen Herstellung
Additif détergent-dispersant pour huiles lubrifiantes pour moteur à combustion interne et son procédé de préparation

(30) Priority: 15.04.1994 HU 9401100
(43) Date of publication of application: 18.10.1995
(73) Proprietor: MOL MAGYAR OLAJ ES GAZIPARI RESZVENYTARSASAG, H-1051 Budapest (HU); VESZPREMI EGYETEM, H-8201 Veszprém (HU)
(72) Inventor: Dénes, Ferenc Dr., H-2921 Komárom (HU); Kis, János, H-2931 Almásfüzitö (HU); Baladincz, Jenö, H-2900 Komárom (HU); Auer, János, H-2903 Komárom (HU); Deák, Gyula Dr., H-4400 Nyiregyháza (HU); Bartha, Laszlo Dr., H-8200 Veszprém (HU); Hancsok, Jenö Dr., H-8200 Veszprém (HU); Kovács, Magda Dr., H-8200 Veszprém (HU)
(74) Representative: von Füner, Alexander, Prof.h.c. Dr.

(56) References cited:
- EP-A- 0 002 286
- EP-A- 0 031 236
- EP-A- 0 145 235
- EP-A- 0 355 895
- EP-A- 0 400 866
- WO-A-88/07557
- GB-A- 2 102 813
- US-A- 161 452
- US-A- 440 659
- US-A- 4 036 772

## Description

The present invention particularly relates to a grafted polyisobutylene - polysuccinic anhydride based ashless detergent dispersant (DD) additive that increases both viscosity and viscosity index and which can be used advantageously for improving the properties of lubricating oils and to a process for the preparation thereof. The ashless, imide and ester type additives synthesised from alkenyl-succinic acid derivatives have been used for more than thirty years for the improvement of the detergent - dispersant properties of motor oils. Due to their polar and often basic character these additives restrict the formation and surface deposition of the insoluble acidic contaminations formed during the operation of the engine. Thus the life span of the engine and the duration of applicability of oils are significantly increased.

The various, so called, modified derivatives containing sulfur, boron, halogens, molybdenum, copper atoms etc. exhibit good anticorrosion and antiwear properties beside their DD effect, whereas those containing large molecular weight ($\overline{\text{M}}$ₙ > 2000) polymer side chains impart viscosity and viscosity index improving properties.

The alkenyl-succinic acid derivatives are generally mixed into the lubricating oils together with other metal containing DD additives, with VI improvers, antioxidants, anticorrosion and antiwear components, friction modifiers and foam inhibitors making use of advantageous interactions.

In the last ten years, the manufacturers of oil additives directed their research to improve the DD efficiency and the advantageous by-effects. According to results of engine tests this can be achieved either by increasing the molecular weight of the intermediates and the end product, or by the formation of polysuccinimides, polyesters, polyester-amides etc. coupled through their polar groups (e.g. U.S. Patent No.4.234,435).

The synthesis of such additives is based on the recognition that in the first step of the succinimide synthesis when the polyolefins and the maleic anhydride (MAH) are reacted under specific conditions more than one MAH is coupled to the polyolefin molecule or alternatively the so called olefin - MAH copolymers are formed. When the so formed intermediates having more than two carboxylic groups are reacted with amines, polyamines, alcohols, polyalcohols, alkanolamines or their mixtures of various compositions then higher molecular weight polyimide, polyamide, polyester, polyester-amide type end products are obtained (e.g. U.S. Patent No. 4.234,435).

Despite of their high DD effect, these ashless additives have only a low base number due to the blocking of their basic amino and imino groups and compared to the traditional succinimides they cause less damage to the fluor containing elastomer sealings of the engines.

Owing to the higher DD effect and significant viscosity and viscosity index increasing effect of these ashless additives they increase the performance level of the engine oils and proved also to be useful in replacing a part of the traditional additives used for improving flow properties reducing thereby the costs of motor oil production. In the published procedures various methods are recommended for the synthesis of the alkenyl-succinic anhydride type intermediates.

According to US 4.234.435 and EP 0.208.560 the succinic anhydride (SA) : polyisobutylene (PIB, $\overline{\text{M}}$ₙ = 1300 - 5000) molar ratio can be increased over 1.05 by a one or multi step addition of the chlorine catalyst and by raising the temperature up to 160 - 220 °C. A serious disadvantage of this process is that hazardous chlorine is built in the polyolefin molecule during the addition reaction, and referred to the additive, it remains in the end product in a 0.001 - 0.5 weight percent.

Processes have also been reported where the polyisobutylene -MAH addition is achieved at high temperature (over 190 °C) without the use of a catalyst. SA/PIB molar coupling ratios higher than one have been achieved by using highly reactive (more than 70 percent alpha olefin content) polyisobutylene raw material and a large excess of MAH. The disadvantages of this method are the need for a more expensive raw material, the high reaction temperature and the long reaction time (e.g. European Patent No.0.271.937.).

A low temperature process has been reported in the WO 90/03359 where the polyisobutylene - maleic anhydride copolymer was prepared by using a radical initiator and an aromatic or chlorinated hydrocarbon solvent. In the PIB-MAH copolymer of alternating structure the average number of the PIB-MAH units varies from 1.1 to 20. When these type of intermediates are used for the acylation reaction then the end products might have a wide range of molar weight ($\overline{\text{M}}$ₙ = 10 000 - 150 000).

EP 0 400 866 discloses an oil-soluble composition useful as a multifunctional viscosity improver additive for oleaginous composition comprising adduct of:
(A) high molecular weight ethylene copolymer substituted carboxylic acid material comprising reaction product of (i) ethylene copolymer having a number average molecular weight of at least 15,000, and (ii) monounsaturated carboxylic acid material; and
(B) at least one polyamine containing one primary amino group and at least one secondary amino group.

Furthermore, EP 0 400 866 discloses an embodiment of said composition which comprises reaction product of (A), (B) and (C) a C₅₀ to C₄₀₀ hydrocarbyl substituted carboxylic acid component containing 1 to 2 carboxylic acid groups or anhydride group.

EP 0 002 286 generally discloses an oil-soluble graft copolymer, suitable for use as an additive for lubricating oils and liquid hydrocarbon fuels, comprising substantially linear, substantially saturated, rubbery, olefinic hydrocarbon backbone polymer and graft polymerized thereon, copolymerized units of a monomer system comprising maleic acid and/or maleic anhydride and one or more other monomers copolymerizable with maleic acid or maleic anhydride, said copolymerized units being post-reacted with a polyamino compound containing one primary or secondary amino group or one primary amido group.

According to EP 0 002 286, suitable backbone polymers include ethylene/propylene copolymers, ethylene/propylene/diene modified terpolymers, hydrogenated styrene-butadiene copolymers, styrene-isoprene copolymers and atactic polypropylene.

Concerning the selection of backbone polymer molecular weight it is stated in said document that the lower molecular weight starting backbone polymer materials are more difficult to handle since they are semi-liquids or exhibit cold flow at ambient temperature (about 20°C), and it is often difficult or uneconomical to control molecular weight during graft copolymerization. While use of a low molecular weight starting polymer may avoid the need for subsequently degrading the graft copolymer product, the difficulty of handling and processing such starting polymers tends to override any such advantage. Accordingly, it is preferred to use a somewhat higher molecular weight starting backbone polymer, of the order of at least about 100,000 viscosity average molecular weight, to avoid such problems.

The methods published so far for the advantageous synthesis of the high molecular weight polyfunctional succinimides have both technological and structural limitations.

According to the advantageous examples patented for the synthesis of the polyisobutylene based succinimides the use of polyisobutylene of average molecular weight $\overline{\text{M}}$ₙ = 1300 - 2500 can be considered as typical and beneficial. As it is well known, the increasing of the average molecular weight of the polyisobutylene raw material above the limit of $\overline{\text{M}}$ₙ = 2500 leads to considerable difficulties in the traditional technologies due to the high viscosity of the raw material. In addition to this, experience shows that due to the application of these raw materials a significant disadvantageous increase of the cold viscosity and a decrease of the polar nitrogen containing groups per unit mass of the additive and a concomitant decrease in the DD effect can be expected.

Succinimide derivatives obtained by grafting of ethylene - propylene copolymers have been produced and applied to achieve an additional DD effect beside their main viscosity and viscosity index increasing functions (EP 400866, EP 002286). For these kind of additives the optimal viscosity and viscosity index increasing effect occurs in the molecular weight range of $\overline{\text{M}}$ₙ = 15000 - 200 000. Successful application of olefin copolymers of a number average molecular weight lower than 15 000 have not been reported probably due to a loss in their flow property improving effect.

Surprisingly, however, it has been recognised that by making use of our invention polyisobutylene based succinimide additives with significant DD, viscosity and viscosity index increasing properties can be synthesised even in the molecular weight range deemed unfavourable for both the polyisobutylene and the ethylene-propylene copolymers.

The invention is based on the recognition that the mentioned drawbacks of the synthesis based on grafting the hydrocarbon polymers limiting the average molecular weight of the applicable raw material can be eliminated by the appropriate control of the grafting reaction. The recommended procedure makes feasible the synthesis of such intermediates from polyolefins of lower average molecular weight and in addition to this the intermediates obtained from polyisobutylenes or especially from their high alpha-olefin containing so called high reactivity homologous are suitable for the preparation of additives of new molecular structure showing higher viscosity and viscosity index improving effect, more advantageous antifriction effect and at the same time exhibit a better compatibility with the sealing materials as compared to the other well known ashless dispersants of molecular weight lower than 15 000.

A subject matter of the invention is an additive for use in an oil solution in lubricating oils of internal combustion engines, which contains imides and/or esters and/or ester amides of the reaction product of a polyisobutylene of a number average molecular weight from 800 - 15 000, an unsaturated reactive dicarboxylic acid and/or its anhydride, preferably maleic anhydride, and another low molecular weight unsaturated comonomer,
wherein said reaction product contains on the average 1.6 - 6.0 dicarboxylic acid and/or its anhydride, preferably succinic anhydride groups per polyisobutylene chain,
in said reaction product the concentration of molecules containing more than one dicarboxylic acid and/or its anhydride, preferably succinic anhydride groups is more than 25%,
the widening of the molecular weight distribution of said reaction product is less than 70 percent, referred to the starting polyisobutylene,
and in said reaction product the polyisobutylene is grafted on or reacted with a dicarboxylic acid and/or its anhydride, preferably succinic anhydride containing copolymer formed from a low molecular weight unsaturated comonomer of a molecular weight less than 500, or from a mixture of such comonomers, and from an unsaturated reactive dicarboxylic acid and/or its anhydride, preferably maleic anhydride, using a molar ratio of 1.2 - 5.5 : 0.1 - 3.5 : 1 of dicarboxylic acid and/or its anhydride, preferably maleic anhydride : comonomer : polyisobutylene,
and the imides and/or esters and/or ester amides of said reaction product are obtained by reacting the dicarboxylic acid and/or its anhydride, preferably succinic anhydride groups, of the copolymer linked to the polyisobutylene in a 0.7 - 5.5 ratio with at least bifunctional compounds containing one or more amine and/or hydroxyl groups.

A further subject matter of the invention is a process for preparing a detergent - dispersant additive, wherein a dicarboxylic acid and/or its anhydride, preferably maleic anhydride, and another low molecular weight comonomer with an olefinic double bond or a mixture of such comonomers and/or a copolymer of a low degree of polymerization prepared previously and consisting of unsaturated dicarboxylic acid and/or its anhydride and the comonomer and/or comonomers are grafted to or reacted with a polyisobutylene of an average molecular weight from 800 - 15 000 by an addition reaction using the molar ratio 1.2 - 5.5 : 0.1 - 3.5 : 1 of dicarboxylic acid and/or its anhydride, preferably maleic anhydride : comonomer : polyisobutylene, where the solvent concentration providing homogeneous phase is 10 - 75 weight percent, preferably 35 - 60 weight percent with respect to the reaction mixture, carried out in the presence of 5 - 25 weight percent of a radical initiator and of 0.01 - 5 weight percent, referred to the dicarboxylic acid and/or its anhydride, preferably maleic anhydride, of a monomer incorporation ratio controlling component at 1 - 15x10² kPa pressure and preferably in nitrogen and/or hydrocarbon atmosphere, at 80 - 180° C, in 1 - 16 hours while the concentration of the dicarboxylic acid and/or its anhydride, preferably maleic anhydride and the comonomer is kept below 5 weight percent, the obtained intermediate is stripped off from its solvent content and is diluted with refined base oil, if desired, and when it is necessary it is clarified and filtered in the presence of a filtration aid, the intermediate is reacted with at least bifunctional compounds containing one or more amine and/or hydroxyl groups, while the ratio of the compounds carrying the dicarboxylic acid and/or its anhydride, preferably succinic anhydride groups and the amine and/or hydroxyl groups is 0.7 - 5.5, wherein the reaction is carried out at 0.05 - 6x10² kPa pressure, at 120 - 235° C, in 2 - 15 hours and optionally in the presence of a catalyst in 0.1 - 2 weight percent referred to the reaction mixture, and the product, if desired, is modified in a usual way, diluted and filtered.

Polyisobutylenes of a number average molecular weight between 1300 and 8000 were found to be the most advantageous.

Today, these kind of polyisobutylenes, especially of average molecular weight above 5000, have some limited applications as viscosity and viscosity index improving additives. Despite of their good thermal oxidation and shear stability their widespread application is limited because they increase the low temperature viscosity of the oils more than other type of viscosity index improving polymers. For this reason they cannot be applied alone in the production of modern multi-grade motor oils. The method according to the invention dramatically decreases and in preferable cases eliminate these disadvantages of the PIB based viscosity index improving additives. Grafting the polar side chain into the PIB main chain results in a combined polymer structure having good thermal and chemical stability as well as viscosity increasing effect characteristic of polyisobutylenes, and at the same time the cold viscosity increasing effect is decreased significantly due to a decrease in the solubility of the polymer.

As comonomers reactive, polar and apolar monomers of low molecular weight such as ethylene, propylene, butene-1, 1,3-butadiene, isobutylene, C₅₋₂₀ alpha olefins, styrene, acrylic acid, methacrylic acid, acrylates and methacrylates prepared from alcohols of C₁₋₂₀, acrylonitrile or their mixtures have been applied.

The polyisobutylene - polysuccinic acid products prepared from polyisobutylene, unsaturated dicarboxylic acid and/or its anhydride and from comonomer or from comonomer mixture having the general formula I. where:
- R: is a polyisobutylene ($\overline{\text{M}}$= 800 - 15 000),
- n: is an integer from 1 to 4, preferably 1,
- m: is an integer from 0 to 5, preferably 1,
- p: is an integer from 1 to 15, preferably from 2 to 6.
- Y: means: and/or a group containing less than 30 carbon atoms, formed from another olefin or diolefin or a mixture thereof,
- X: stands for hydrogen or a saturated or unsaturated group formed from Y group, and
- R₁ and R₂: stand for hydrogen or C₁₋₂₀ alkyl group.

Those derivatives are the most suitable where the number of the succinic anhydride (SA) groups linked to one polyisobutylene molecule is between 1.6 and 6 on average, preferably between 1.8 and 4 on average, and the concentration of the molecules containing more than one SA group is at least 25 weight percent, the concentration of the free maleic acid is less than 0.3 weight percent and the increase of the number average molecular weight of the components determined by GPC is smaller than 2.5 times the molar weight of the starting polyisobutylene. The intermediate consisting of the above long apolar polyisobutylene chain and a shorter, strongly polar, random or alternating copolymer chain is especially suitable for the preparation of the imide and/or ester and/or amide and/or ester-amide derivatives of great dispersing effect, where the derivatives occurring in one polyisobutylene chain could be identical or different.

It is also ensured by the multifunctional usually polar chain terminating groups that by using appropriate at least bifunctional basic reagents in the acylation reaction additives of chain like polymers are formed under advantageous conditions beside the usual crosslinked polymers.

The additive prepared according to this invention could contain components of various average molecular weight in which the average number of molecules linked by the carboxyl groups is between 2 and 100.

The additive prepared according to this invention is used advantageously in an oil solution. In this oil solution the concentration of the oil is at least 10 weight percent, preferably between 30 and 80 weight percent. For this purpose any type of refined oil, lubricating oil or base oil may be used.

In the actual preparation procedure maleic anhydride and comonomer or comonomers containing olefinic double bond or their copolymers are grafted to the starting polyisobutylenes. During the reaction the double bonds of the maleic anhydride and the comonomer or the comonomers are activated by a radical initiator and due to the consecutive coupling to the polyisobutylenes and/or due to the coupling of the random or alternating copolymers formed from the maleic anhydride and a comonomer a polymer chain is developed containing several SA groups (general formula I.).

The first step of the synthesis of the additive i.e. the reaction of the polyisobutylene and the unsaturated dicarboxylic acid and/or its anhydride, preferably maleic anhydride and comonomer or comonomers is performed in a homogeneous solution at an energetically favourable low temperature, with the suitable choice of the weight ratio corresponding to the molar ratio of the reactants of various reactivity, under circumstances unfavourable for the multiple coupling of the polyisobutylene occasionally in the presence of compounds controlling the structure of side chain containing polar groups.

The reaction of the polyisobutylene and the unsaturated dicarboxylic acid and/or its anhydride preferably maleic anhydride and the comonomer or the comonomers was carried out in a solvent containing components also within the boiling range of 110 - 250 °C and in which the reactants and the intermediates were readily dissolved at a concentration of 20 - 75 weight percent, preferably 35 - 60 weight percent with respect to the reaction mixture, in the temperature range 80 - 180 °C, preferably between 120 - 160 °C, within a reaction period of 1 - 16 hours, using 1.2 - 5.5 : 0.1 - 3.5 : 1 maleic anhydride : comonomer : polyisobutylene molar ratio, and applying 5 - 25 weight percent peroxide, with respect to the amount of maleic anhydride, or other type of initiator such as azobisisobutyronitrile or cumene hydroperoxide or if desired, compounds or their mixtures controlling the incorporation ratios of the monomers in 0.01 - 5 weight percent, with respect to the amount of the maleic anhydride, at a pressure of 1 - 15x10² kPa, preferably at 1 - 5x10² kPa, in an inert atmosphere such as nitrogen and/or hydrocarbon gas.

It has been found that high SA/polyisobutylene average molar ratio can be achieved, while the formation of the oil insoluble by-product is kept at a minimum level, if such a solvent or a mixture of solvents is used wherein the fraction of components having a boiling point below 250 °C is at least 3 weight percent. In order to decrease the concentration of by-products insoluble in oil the concentration of the comonomer or the comonomers should be less than 5 weight percent in the reaction mixture during the addition. These conditions can be met if the rates of addition of the MAH, the comonomer or the comonomers and the radical initiator decomposing in the temperature range 80 - 180 °C are set to appropriate values. For this purpose the radical initiator, the MAH as well as the comonomer or the comonomers are added in two or more portions or in a continuous way.

As initiator, organic peroxides, hydroperoxides or azo- compounds such as dibenzoyl peroxide, di-tert-butyl peroxide, azobis-isobutyro dinitrile, azodicarboxylic amide, or their mixture can be used.

Compounds used for inhibiting undesirable side reactions, such as e.g. decarboxylation, resin formation, or for controlling the MAH : comonomer incorporation ratio could be carboxylic acids with 1 - 20 carbon number, dicarboxylic acids or anhydrides, hydroxycarboxylic acids, ketones, ethers, esters, alcohols, water or the mixtures of these and their derivatives. Isobutyl alcohol, isopropyl alcohol, succinic monobutyl ester can be applied advantageously. If desired, such additives are applied in a concentration of 0.01 - 5 weight percent with respect to the amount of the maleic anhydride. During the decomposition of these compounds or the radical initiators highly reactive species may be formed that may participate in the addition and polymerisation reactions occurring in the reaction mixture.

The reaction products have been identified by their ¹³C and ¹H NMR spectra using deuterated chloroform as solvent. It has been pointed out that under the experimental circumstances applied in this invention the monomers added to the reaction mixture are mostly coupled to the α-double bond of the polyisobutylenes. This has been proved by the disappearance of the ¹³C peaks at 114.5 and 143.6 ppm characteristic of the terminal double bonds of the polyisobutylenes, as well as the peaks of the ¹H spectra at 4.3 ppm and of the ¹³C peaks at 136.6 ppm typical of the maleic anhydride and of the peaks characteristic of the double bonds of the comonomers. Experiments with maleic anhydride enriched in ¹³C isotope proved the existence of bonds characteristic of the built in comonomer groups forming the grafted copolymer chains.

From the colourless - light brown intermediate prepared according to this invention the solvent can be recovered by stripping out the components of a boiling point below 250 °C and the remaining heavier part, if desired, can be diluted in 20 - 60 weight percent by refined oil, preferably by a refined oil having viscosity of 2 - 15 mm²/s, at 100 °C.

The solution of the intermediate can be filtered without or with the addition of a filtration aid or filtration improving material in a 0.5 - 5 weight percent concentration.

If the intermediate prepared according to this invention is reacted in the second so called acylation step with polyamines, polyalcohols, alcanol amines containing at least two reactive groups and/or their mixtures and/or their derivatives by using hydrocarbon and/or refined oil as solvent at 120 - 235 °C, in inert e.g. nitrogen gas atmosphere at a pressure of 0.05 - 6x10² kPa, in the presence of a catalyst in a 0.01 - 2 weight percent concentration then a polysuccinimide and/or polyamide and/or polyester and/or polyester-amide based mixture of the additive is obtained (such as the polysuccinimide, general formula II.) where one or more components can be formed with significantly different molecular weights depending on the reagents and molar ratios used. where:
R is a polyisobutylene group (molar weight = 800 - 15 000),
U stands for an at least bifunctional group derived from polyalkylene - polyamines and/or polyalcohols and/or polyalkanolamines or other usual compounds containing basic nitrogen and/or hydroxyl group,
Y' means a: group, or another bifunctional group formed from an olefin or diolefin or a mixture thereof, or a monofunctional group obtained by transformation of the groups defined above,
Z means hydrogen or -NH-(CH₂CH₂NH)-H or -OR₁ group,
R₁ and R₂ stands for C₁₋₂₀ alkyl group each,
a,b,c,d,e and f are integers from 0 to 5, preferably 1,
q,m,n are 0, 1 or an integer greater than 1, with the proviso that:
the sum of m and n is an integer greater than 1, the proportion of molecules containing groups (II.b) and/or (II.c) in the product is higher than 25 % by weight and the compounds of structures (II.a), (II.b) and (II.c) can be interconnected in an optional sequence.

The important feature of the additive prepared according to this invention is due to the new structure of the intermediate. In this intermediate the presumably reactive SA and other groups are closely located at the end of the long polyisobutylene chain. Consequently, the growing of the macromolecule by multiple or chain like coupling is not hindered sterically, as in the case of other intermediates where the SA groups are randomly located either at the end or in between the polyisobutylene chains.

As a multifunctional polyamine component e.g. ethylene- diamine, diethylenetriamine, triethylenetetramine, tetraethylenepentamine, pentaethylenehexamine, cyclic polyamine e.g. piperazine, diethyleneamino piperazine or the mixtures of these; as polyalcohol e.g. ethylene glycol, diethylene glycol, triethylene glycol, glycerol, trimethylol propane or pentaerythritol; as amino-alcohol e.g. ethanolamine, diethanolamine, triethanolamine, or the mixtures and derivatives of these can be used.

Since in the additive the mole fraction of the various polymers of different molar weights can be altered in a wide range the need to prepare different motor oils is met easily by a slight modification of the preparation procedure.

According to our experience, especially those additive compositions proved to be advantageous where, in terms of weight percentage, the higher molar weight / lower molar weight ratio was in the 0.01 - 5 range.

The average molecular weight of the lower average molecular weight polymer is less than six times the number average molar weight of the polyisobutylene used as raw material. The experimental circumstances of the acylation have to be chosen in such a way as to promote the formation of multiple couplings in the amide, imide and ester formation condensation reactions, i.e. that result in compounds characterised by polyamide, polyimide and polyester structure or by their combination. This can be achieved by keeping the molar ratio of the succinic anhydride group of the intermediate and the component to be acylated in the 0.7 - 5.5 : 1 range, preferably in the 1.7 - 4.5 : 1 range.

In order to ensure the required level of conversion in the acylation a 2 - 15 hour reaction period and, if desired, the usual acidic or basic catalysts were used in a 0.1 - 2 weight percent concentration range.

As a catalyst, acidic or basic compounds such as petroleum sulfonic acid, p-toluenesulfonic acid, sulfuric acid, potassium hydroxide, triethanolamine, ethanolamine or ion exchange resin, preferably in hydrogen ion form can be used in the acylation reaction.

In the polyester formation, which is one possible version of the acylation, the petroleum sulfonic acid can be used especially advantageously which so far has been suggested as a catalyst only in the preparation of low molecular weight ($\overline{\text{M}}$ₙ < 3500) alkenyl succinic esters (Hungarian Patent No. 205.778).

After the acylation reaction the non-reacted acid can be removed, if this is needed. In order to promote other preferential by-effects such as the anticorrosion or anti-wear, antioxidant effect a structure modifying step can be applied as a finishing one. In this process a modifying compound is added in a 0.1 - 8 weight percent concentration referred to the reaction mixture, which is then stirred for 0.5 - 10 hours, at 80 - 230 °C temperature, in inert atmosphere.

For modification the usual modifying chemicals can be applied, such as sulfur, active sulfur containing compounds, phosphorus pentasulfide, boric acid or its derivative, zinc containing compounds like zinc dialkyldithiophosphate, copper compounds including organic copper salts or complexes, molybdenum dioxide, organic acids e.g. fatty acids, glycolic acids, malic acid, fumaric acid, amides, alkenyl succinimide, their mixture or their derivatives.

After the completion of the acylation and the optional modifying reactions the volatile components can be stripped off from the reaction mixture in vacuum, at 160 - 210 °C, the reaction product is then diluted by refined oil, and if desired, it can be filtered without or with the use of filtration aids.

The various components of different average molecular weight of the end product exhibit characteristic differences, the additives containing the lower molecular weight components in a higher concentration have a higher acid neutralising capacity and deposition removing effect, whereas the products containing the higher molecular weight components in a higher concentration have a significant dispersion stabilising, viscosity and viscosity index increasing as well as an anti-wear effect.

In the products described herein the components are characterised by their number average molecular weight calculated as follows:${\overline{\text{M}}}_{\text{n}} \text{=} \frac{\text{Σ} {\text{n}}_{\text{i}} {\text{M}}_{\text{i}}}{\text{Σ} {\text{n}}_{\text{i}}}$ where
$\overline{\text{M}}$ₙ is the number average molecular weight,
nᵢ is the mole number of the i-th polymer molecule,
Mᵢ is the molar weight of the i-th polymer molecule,
i is 1,2,... positive integer.

The degree of polydispersity characterising the molecular weight distribution is the ratio of the weight average and number average molecular weights. The weight average molecular weight is calculated by the following equation:${\overline{\text{M}}}_{\text{w}} \text{=} \frac{\text{Σ} {\text{n}}_{\text{i}} {\text{M}}_{\text{i}} {\text{}}^{\text{2}}}{\text{Σ} {\text{n}}_{\text{i}} {\text{M}}_{\text{i}}}$ where $\overline{\text{M}}$_{w} is the weight average molecular weight, the other symbols have the same meaning as above. Polydispersity is calculated by the following equation:$\text{α =} \frac{\overline{{\text{M}}_{\text{w}}}}{\overline{{\text{M}}_{\text{n}}}}$ The widening of the molecular weight distribution (Δα) is:$\text{Δα =} \frac{{\text{α-α}}_{\text{PIB}}}{{\text{α}}_{\text{PIB}}} \text{· 100}$ where α_{PIB} is the polydispersity of the polyisobutylene raw material and α is the polydispersity of the reaction product.

The invention is illustrated by the following non-limiting examples.

### Example "A"

In a 3 dm³ pressure proof, stirred tank reactor equipped with thermometer, inert gas supply and a cooler on the top connected to a condensate collecting vessel 1125 g (0.5 mole) polyisobutylene ($\overline{\text{M}}$ₙ = 2250) and 1450 g xylene is weighed, the mixture is heated to 76 ± 4 °C in inert atmosphere and under stirring, 98.6 g (1 mole) maleic anhydride, and at a rate of 0.7 g/h 2.8 g dibenzoyl peroxide are added and altogether 28 g isobutylene in four portions, 7 g each. After the completion of additions the reaction mixture is stirred for an hour under the above conditions. The xylene and other unreacted lighter components can be removed by distillation carried out at 140 °C, at 15 kPa pressure, for 1.5 hours. 1200 g refined lubricating oil (viscosity 3.5 mm²/s at 100 °C, viscosity index 95, pour point -22 °C) is added to the intermediate. After homogenization at 135 - 150°C and clarification the mixture is filtered in the presence of 3.5 weight percent filtration aid. The acid number of the yellow - brown, viscous, oily intermediate is 43.0 mg KOH/g, its maleic anhydride content is 1.5 mg/g and it contains 1.7 succinic anhydride group on the average referred to a PIB molecule. The SA/PIB succination ratio was calculated by the following equation:$\text{SR} \text{=} \frac{{\overline{\text{M}}}_{\text{nPIB}} \text{·} \text{E}}{{\text{112.2 · 10}}^{\text{3}} \text{- 98.6 ·} \text{E}}$ where
SR = SA/PIB succination ratio,
E = acid number of the intermediate (mg KOH/g),
$\overline{\text{M}}$_{nPIB} = number average molar weight of the PIB.

### Example "B"

The reaction vessel described in Example "A" is charged with 1125 g (0.5 mole) polyisobutylene of a number average molar weight, $\overline{\text{M}}$ₙ = 2250, 950 g SAE-30 base oil (viscosity 9.5 mm²/s at 100 °C) and 110 g of MOL Rt. solvent of high aromatic content (having the trade name AROMATOL) and mixed. The mixture is stirred at atmospheric pressure in inert atmosphere, at 135 ± 6 °C and in 8 equal portions 118.3 g MAH, 76 g octylmethacrylate and 9.6 g di-tert-butyl peroxide are added to it in 4 hours. The reaction mixture is then stirred for further 6 hours and the AROMATOL and the other lighter components are boiled off at 155 °C, and 12 kPa pressure. To the intermediate 250 g SN-150/A (MOL Rt.) refined oil is added at 120 °C. The so obtained intermediate is first clarified with 2 weight percent filtration aid and in the presence of 1 weight percent of a filtration improving material it is filtered at 110 °C. The acid number of the diluted and filtered intermediate is 39.7 mg KOH/g, its maleic anhydride content is 2.8 mg/g and it contains 1.6 succinic anhydride group on average referred to a PIB molecule. The increase in the average molecular weight is less than 60 percent and the fraction of the compounds containing more than one succinic anhydride group per molecule is more than 55 percent.

### Example "C"

Into the reaction vessel described in Example "A" 1200 g (0.15 mole) polyisobutylene ($\overline{\text{M}}$ₙ = 8000), and 500 g xylene were weighted and mixed. The mixture was then heated to 115 °C and in six equal portions, in 3 hours 59.2 g (0.6 mole) maleic anhydride, 12.0 g azobisisobutyronitrile and 24.0 g styrene were added. Following the additions the reaction mixture was heated up to 180 °C and was stirred for a further 6 hours. The unreacted maleic anhydride was removed at 195 °C and 10 kPa pressure, the product was then mixed with 1150 g refined lubricating oil mentioned in Example "A" and the obtained mixture was filtered in the presence of 3 weight percent filtration aid. The acid number of the filtered and diluted intermediate is 23.9 mg KOH/g, its maleic anhydride content is 1.3 mg/g and it contains 3.3 succinic anhydride group, on average, referred to a PIB molecule. The increase in the average molecular weight and the widening of the molar weight distribution is less than 20 percent and the fraction of the compounds containing more than one SA group per molecule is 42 weight percent.

### Example "D"

Into the reaction vessel described in Example "A" 1200 g (0.5 mole) polypropylene and a 9 : 1 weight ratio mixture of an SN 150/A base oil (commercial product of the MOL Rt.) and kerosine were added. The mixture was heated to 80 ± 4 °C and under stirring 98.6 g (1 mole) maleic anhydride and 4.2 g di-benzoyl peroxide were added, the mixture was stirred for 2 hours and the temperature was raised to 160 °C and the following components were added to it: 33 g isobutylene; as initiator 11.4 g di-tert-butyl peroxide; in 2 - 2 equal fractions per hour 43.3 g maleic anhydride, 6.5 g succinic monobutyl ester; 33 g styrene and within 6 hours in 5 equal fractions 88.7 g maleic anhydride.

The unreacted, lighter components were removed at 200 °C and at 10 kPa pressure during one and half hour. The product was then diluted with 1060 g of the base oil mentioned in Example "B" and the obtained mixture was filtered in the presence of 4 weight percent filtration aid, the acid number of the filtered and diluted intermediate was 60.1mg KOH/g, its maleic anhydride content was 2.1 mg/g, its average SA : PP succination ratio was 2.4, the fraction of the components containing more than one SA group per molecule was 64 percent, the increase in the average molecular weight was less than 60 percent, and the measured widening of the molar weight distribution was 68 percent.

### Example "E"

Into the reaction vessel described in Example "A" 0.08 mole polyisobutylene ($\overline{\text{M}}$ₙ = 15000) 600 g xylene, 0.4 g cumene hydroperoxide and a 1 : 1 weight ratio mixture of fumaric acid : maleic anhydride mixture were added, the mixture was stirred and heated to 180 ± 5 °C, in inert atmosphere at 6 bar for 2.5 hours. The reaction mixture was then cooled down to 150 ± 4 °C and under stirring 9 g acrylic acid and 1.8 g di-tert-butyl peroxide as well as 12.8 g of the above acid mixture were added in 6 equal fractions in 6 hours in such a way that before each addition of the acrylic acid 0.5 - 0.5 g isobutyl alcohol was also added to the mixture. After the distillation carried out for two hours at 165 °C and 15 kPa pressure, 1000 g oil characterised in Example "A", 2 - 2 percent filtration aid and filtration improving material were added and was filtered. The acid number of the filtered and diluted intermediate was 9.3 mg KOH/g, its maleic anhydride content was 1.7 percentage, its average dicarboxylic acid - polyisobutylene coupling ratio was 2.3, the fraction of the compounds containing more than one group originating from the dicarboxylic acid was 47 percent, the increase in the average molecular weight and in the widening of the molar weight distribution were less than 10 percent.

### Example "F"

Into the reaction vessel described in Example "A" 500 g xylene saturated with water and 28.5 g isobutylene were weighed and under stirring the mixture was heated to 130 ± 5 °C in 2 hours, 0.75 mole (73.95 g) maleic anhydride and under continuous feed 14 g di-tert-butyl peroxide initiator was added, at 130 °C, to this reaction mixture 3 g succinic monobutyl ester were added in drops in half an hour, after about 0.25 hours 98.6 g maleic anhydride, 60 g styrene and 27 g di-tert-butyl peroxide initiator were added in 4-4, and the latter in 6 equal fractions. Before the addition of the last two fractions of the initiator 0.5 mole poly-isobutylene ($\overline{\text{M}}$ₙ = 2250) and 0.5 mole (43.3 g) maleic anhydride were added to the reaction mixture which was then heated to 140 ± 5 °C and stirred for 1 hour. The unreacted, lighter components of the mixture were removed by boiling for 1.5 hours at 175 °C and at 15 kPa pressure. The product so obtained was then diluted with 1200 g of the base oil mentioned in Example "B" and was filtered in the presence of 2 weight percent filtration improving material. The saponification number of the filtered and diluted intermediate was 78.8 mg KOH/g, its maleic anhydride content was 1.9 mg KOH/g, its average SA : PIB succination ratio was 3.1, the increase of the average molecular weight was less than 30 percent, the widening of the molar weight distribution was 40 percent, the fraction of the components containing more than one succinic anhydride group per molecule was 65 percent.

### Example " G "

Into the reaction vessel described in Example "A" 800 g SN 150/A base oil and 200 g xylene saturated with water were weighed and through this mixture 10 g " C₄ - fraction" (product of naphtha pyrolysis, commercial product of the TVK Rt.) was bubbled through and under stirring the mixture was heated to 90 ± 3 °C with a rate of 50°C/hour and in 2 hours, 0.5 mole (49.3 g) maleic anhydride and 12 g dibenzoyl peroxide were added in 3 - 3 equal portions, the temperature of the reaction mixture was then raised to 140 ± 5°C and in 4 hours 70 g styrene, 147.9 g (15 mole) maleic anhydride and 14 g di-tert-butyl peroxide were added in a continuous way. To the oily xylene solution of the low molecular weight copolymer 1125 g (0.5 mole) poly-isobutylene was added and the reaction mixture was then heated to 140 ± 5 °C and under continuous stirring for 1 hour 10 g di-tert-butyl peroxide was added, the mixture was then stirred for a further 1.5 hours. The unreacted, lighter components of the mixture were removed by boiling as in Example "A" and the obtained intermediate diluted further by 300g SN 150/A oil was suitable for further use without filtering and further processing. Its acid number was 72.4 mg KOH/g, maleic anhydride content was 1.8, its average SA : PIB succination ratio was 3.3, the increase of the average molecular weight was less than 35 percent, the widening of the molar weight distribution was 45 percent, the fraction of the components containing more than one succinic anhydride group per molecule was 73 percent.

### Example " H " (Reference)

Into the reaction vessel described in Example "A" 1125 g (0.5 mole) polyisobutylene and 500 g xylene were weighed. The mixture was heated to 135 ± 5 °C , and in inert atmosphere, under stirring, in 5 equal fractions 111.0 g (1.1 mole) maleic anhydride and in 7 equal fractions 9 g di-tert-butyl peroxide initiator were added. The lighter components of the mixture were removed as in Example " A " and the obtained intermediate was diluted by 1300 g of the oil mentioned in Example " B " , its acid number after clarification and filtration was 31.6 mg KOH/g, its free maleic anhydride content was 3.2 mg/g, the increase of its average molecular weight was less than 15 percent, the widening of the molar weight distribution was 45 percent, the average SA : PIB molar ratio was 1.3 the fraction of the components containing more than one succinic anhydride group per molecule was 35 percent.

### Example " I "

Into the reaction vessel described in Example "A" 950 g (1 mole) polyisobutylene and under stirring in inert atmosphere at 180 ± 10 °C, 270 g of an isobutylene - styrene mixture (weight ratio 4 : 5), in 5 hours, in 5 equal fractions 246.5 g (2.5 mole) maleic anhydride and in 7 hours 28 g di-tert-butyl peroxide were added. After the first hour of the reaction but before all the maleic anhydride has been added 1 - 1 g of isopropyl alcohol was also added in drops to the reaction mixture. The lighter unreacted components of the mixture were removed as in Example " B " and the obtained intermediate was diluted by 1300 g of the base oil mentioned in Example " B ". Its acid number after clarification and filtration again according to Example " B " was 87.6 mg /g, its free maleic anhydride content was 3.0 mg/g, the average SA : PIB succination ratio was 1.5; the increase of its average molecular weight was 60 percent, the widening of the molar weight distribution was less than 68 percent, the fraction of the components containing more than one succinic anhydride group per molecule was 47 percent.

### Example " J " (Reference)

Into the reaction vessel described in Example "A" 1300 g (1 mole) polyisobutylene and 350 g xylene were weighed and under stirring the mixture in inert atmosphere at atmospheric pressure it was heated to 145 °C and in 6 hours, 197.2 g (2 mole) maleic anhydride as well as 11.9 g cumene hydroperoxide and 6.8 g di-tert-butyl peroxide were added in 4 and 7 fractions. The unreacted, lighter components of the mixture were removed by boiling for 1 hour at 150 °C and at 15 kPa pressure. The mixture of the intermediate so obtained was then diluted with 1150 g of the oil mentioned in Example "A" and was filtered in the presence of 3 weight percent filtration improving material. The saponification number of the filtered and diluted intermediate was 70.3 mg KOH/g, its maleic anhydride content was 2.5 mg/g, its average number of the succinic anhydride groups linked to one PIB molecule was 1.6. The fraction of the components containing more than 3 succinic anhydride groups per molecule was 34 percent, the increase of the average molecular weight was 550 percent, the widening of the molar weight distribution was 85 percent referred to the polyisobutylene used as raw material.

### Example " 1. "

In a stirred tank reactor equipped with reagent supply, condenser, sampling facility, nitrogen discharge vent, thermometer and pressure gauge 783.3 g of the acylation reagent described in example " A " is weighed at 65 °C and to this 14.2 g tetraethylenepentamine as well as 0.1 weight percent triethanolamine as catalyst were added. The reaction mixture was then heated to 175 - 180 °C, under stirring in inert atmosphere and the acylation reaction was then continued under such circumstances for 5 hours. This was followed by the addition of 3.1 g diethylenetriamine to the reaction mixture and at 190 °C, at 50, 30 and 10 kPa pressures the mixture was stirred for 1 - 1 hour. The nitrogen content of the end product was 0.8 percent, the ratio of the higher and lower molecular weight polymers was 0.6.

### Example " 2. "

Into the stirred tank reactor described in Example " 1 " 84.7 g acylation reagent characterised in Example " B " and 5 g triethylenetetramine, 22.4 g triethanolamine were weighed at 60 °C . The reaction mixture was then heated to 175 - 180 °C, under stirring in inert atmosphere and the acylation reaction was then continued under such circumstances for 6 hours. In the last four hours of the acylation reaction 300 kPa pressure was applied for 3 hours then for a further hour 10 kPa pressure. After filtration in the presence of 1 weight percent filtration aid the nitrogen content of the obtained product was 0.40 weight percent, the ratio of the higher and lower molecular weight polymers was 0.5.

### Example " 3. "

Into the stirred tank reactor described in Example " 1 " 938.9 g of the intermediate according to Example " C " was weighed at room temperature then at 140 °C, 10.3 g diethylenetriamine was added to it. The acylation reaction was carried out under stirring in inert atmosphere at 50 kPa pressure for 4 hours while the temperature was raised to 190 °C at the rate of 20 °C/hour. After filtration at 120 °C in the presence of 1 weight percent filtration aid the nitrogen content of the obtained product was 0.4 weight percent, the ratio of the higher and lower molecular weight components was 2.3.

### Example " 4. "

Into the stirred tank reactor described in Example " 1 " 746.8 g of the intermediate according to Example " D " , 0.2 weight percent malic acid catalyst and 12.3 g glycerol were added in two parts, at room and at 130 °C temperatures, then the acylation was carried out in inert atmosphere at 210 °C, at 400 kPa pressure for 4 hours, and at 10 kPa for 3.5 hours. The reaction mixture was then cooled down to 120 °C, and 3.1 g diethylenetriamine was added to it, then it was stirred at 155 °C, at 65 kPa pressure for 1 hour, then at 185 °C at 10 kPa pressure for 2 hours. After filtration in the presence of 1 weight percent filtration aid the nitrogen content of the obtained product was 0.11 weight percent, the ratio of the higher and lower molecular weight components was 0.2.

### Example " 5. "

Into the stirred tank reactor described in Example " 1 " 844.5 g of the intermediate according to Example " E " was weighed. Under stirring in inert atmosphere, 1.24 g diethylenetriamine was added at room temperature then at 70 °C 2.27 g tetraethylenepentamine was added and the reaction was carried out for 2 hours at 130 °C. Then a further 0.6 g diethylenetriamine and 1.1 g of tetraethylenepentamine were added in drops to the reaction mixture. The reaction was carried out under atmospheric pressure for 4 hours at 190 °C, and was filtered at 120 °C in the presence of 1 weight percent filtration aid. The nitrogen content of the obtained product was 0.2 weight percent, the ratio of the higher and lower molecular weight components was 0.1.

### Example " 6. "

Into the stirred tank reactor described in Example " 1 " 711.9 g of the intermediate according to Example " F " was weighed and in the presence of 0.2 weight percent petroleum-sulfonic acid catalyst, 6.0 g ethylenediamine was added to this mixture at room temperature and at atmospheric pressure, then the temperature was raised to 190 °C, and the pressure to 15x10² kPa and the acylation reaction was carried out for 6 hours. To the reaction mixture 11.3 g tetraethylene- pentamine was added and at 215 °C, and 10³ kPa pressure the reactants were mixed for 2 hours. After filtration at 120 °C in the presence of 1 weight percent filtration aid the nitrogen content of the obtained product was 0.9 weight percent, the ratio of the higher and lower molecular weight components was 1.25.

### Example " 7. "

Into the stirred tank reactor described in Example " 1 " 774.9 g of the acylation reagent used in Example " G " was weighed, in inert atmosphere, at atmospheric pressure 8.76 g triethylenetetramine and under continuous stirring 9.49 g diethanolamine were weighed. After the acylation reaction carried out at 175 °C under 50 kPa pressure for 4 hours 25 g monosuccinimide derivative (KOMAD-303, MOL Rt.) was added in drops at 120 °C, in 10 minutes. The reaction was continued for 3 hours at 170 °C and 2x10² kPa and for a further 1.5 hour at 15 kPa pressure. The nitrogen content of the obtained product was 0.54 weight percent, the ratio of the higher and lower molecular weight polymers was 0.7.

### Example " 8. " (Reference)

Into the stirred tank reactor described in Example " 1 " 711.3 g of the intermediate prepared according to Example "H" was weighed then in nitrogen atmosphere 10.3 g diethylenetriamine was added at room temperature and at 120°C, 37.8 g tetraethylenepentamine was added and the acylation reaction carried out for 2 hours at 250 °C was followed by the addition of 13.6 g pentaerythritol and 2.4 g of petroleum sulfonic acid as catalyst. After a 3 hours final reaction period at 15 kPa pressure the product was filtered in the presence of 3 weight percent filtration aid. The difficult-to-filtrate product was only partially soluble in base oil due to its 2.2 percent nitrogen content.

### Example " 9. "

Into the stirred tank reactor described in Example " 1 " 768.5 g of the acylation reagent used in Example " I " was weighed, in inert atmosphere, at atmospheric pressure. Under continuous stirring at 80 °C, first 21.2 g diethylene glycol was added in 0.5 hours using a 80 °C/hour heating rate, then 18.9 g tetraethylenepentamine was added in drops to the reaction mixture and the acylation reaction was carried out at 180 °C, under atmospheric pressure for 6 hours. The nitrogen content of the filtered end product was 0.82 weight percent, the ratio of the higher and lower molecular weight components was 0.4.

For the sake of easier handling and comparison - the oil content of all the end products was adjusted to 50 percent before further use. When the oil content of the end product prepared in the various examples was lower than 50 percent then it was adjusted to this value by dilution with the oil component used in the synthesis. For the dilutions refined lubricating oils characterised in Examples " A " and " B " were used.

By comparing the characteristics of the intermediates prepared in Examples " A " to " G " and " I " it turned out that under the circumstances applied in this invention the reaction between the comonomer(s), the polyisobutylene and the MAH leads to the linkage of copolymer chains containing 1.6 - 6, preferably 1.8 - 4 succinic anhydride groups on the average to the polyisobutylene molecule.

The efficiency of the detergent - dispersant effect of the additives mentioned in the above examples was evaluated according to the method described by L.Bartha et al.: Method of determination of optimum composition of detergent - dispersant engine oil additives, Hung. J. Ind. Chem.,1979 7, 359-366. The potential detergent - dispersant effect (PDDE) values are given in terms of percentage as the 225th part of the sum of the dispersion stabilising effect of the additive (detergent index, DI, %) and its washing effect (M, mm). The deposition reducing effect was evaluated by identical methods given in the above quoted publication on the basis of results obtained by the so called panel coking method. In addition to the above characteristics the dispersant effect of the additive has also been evaluated by the so called spot dispersancy test method. According to this method the oil mixture containing the additive or additives to be investigated is mixed in a high speed mixer with 2 percent carbon black of a specific quality and the suspension obtained is treated in six different ways (keeping them at various temperatures, in the presence or absence of water) and from the six suspensions samples are dropped on filter paper and the ratio of the diameters of the carbon black and the oil spots is evaluated after 48 hours. The theoretical maximum of the sum of the six results is 600 percent, the higher the dispersant effect the higher this value.

The detergent - dispersant effect of the products prepared in Examples 1 through 9 were evaluated in lubricating oils and are shown in Table 1.

**Table 1**

| DD efficiency of additive compositions (3 weight percent in an SN-150 oil) | |
|---|---|
| Example No | PDDE, % * (100 max.) |
| Base oil | 1 |
| 1. | 96 |
| 2. | 87 |
| 3. | 76 |
| 4. | 69 |
| 5. | 74 |
| 6. | 85 |
| 7. | 87 |
| 8. | Cannot be evaluated |
| 9. | 86 |

| | |
|---|---|
| * PDDE: potential detergent - dispersant effect | |

For these studies the products prepared according to the mentioned examples were mixed in 3 percent concentration into the base oil characterised by the following parameters:
- Kinematic viscosity (100 °C):: 5.2 mm²/s
- Viscosity index, VI_{E} :: 101

The results of the detergent - dispersant effect studies of the oil compositions obtained using the products prepared in Examples 1.,2.,3. and 7. as well as that of the reference are shown in Tables 2. and 3, while those on viscosity and VI improving are presented in Table 4.

**Table 2.**

| DD properties of oil compositions | | |
|---|---|---|
| Oil compositions * | PDDE, % ** | Deposition on the plate, mg |
| Additive according to: | | |
| Example No.1. | 94 | 3.2 |
| Example No.2. | 92 | 5.7 |
| Example No.3. | 85 | 10.4 |
| Example No.7. | 90 | 14.0 |
| Reference additive | | |
| (KOMAD - 301 ***) | 81 | 9.0 |

| | | |
|---|---|---|
| * Components of the compositions SAE-30 Base oil 91.0 % Additives according to Examples No. 1. or 2.or 3.or 7. 4.0 % Commercially available additives Hyperbasic Ca-sulfonate 3.8 % Zn-dialkyl-dithiophosphate 1.2 % | | |
| ** PDDE: Potential detergent - dispersant effect | | |
| *** Commercially available KOMAD -301 ($\overline{\text{M}}$_{nPIB} = 950; MOL Rt) 4.0 weight percent | | |

**Table 5.**

| Data for the oil compositions obtained by the VW 3344 method | | | |
|---|---|---|---|
| Oil composition | Breaking load, mPa | Breaking elongation % | Storage at 100 % elongation |
| Additive according to: | | | |
| Example No.1 | 9.8 | 225 | Crack free |
| Example No.7. | 9.9 | 215 | Crack free |
| Example No.2. | 11.1 | 271 | Crack free |
| Example No.3. | 11.4 | 269 | Crack free |
| KOMAD-302 | 7.3 | 136 | Broken |
| Minimum level | 8.0 | 160 | Crack free |

Dispersants were studied in the oil compositions shown in Table 3.

The structure and properties of the intermediates prepared according to Examples "A" through "G" and "I" and of the end products synthesised from these according to Examples 1. through 7. and 9. are similar to others prepared according to this invention and were also obtained under the advantageous experimental conditions and parameter combinations of the present invention. The structure and properties of the intermediates and end products according to Examples "H" and "J" as well as 8., and also their preparation are different in some way from the advantageous structures and procedures of this invention.

The results concerning the detergent-dispersant, viscosity modifying, sealing compatibility studies of the end products obtained under advantageous acylation and modifying conditions according to the invention from the intermediates of advantageous structure and composition prepared according to the advantageous conditions of the invention are shown in Tables 1. through 5. and indicate that the efficiency of these products is either identical or superior as compared to the reference additives, i.e. their detergent - dispersant effect in the base oil either in themselves or in oil compositions is really advantageous. Their viscosity index improving effect and their compatibility with sealing materials are significantly superior as compared to commercially available reference additives. The use of additives prepared according to this invention further improves the properties of lubricants or fuels.

Due to their less significant cold viscosity increasing effect the applicable concentration can be further increased especially in the case of motor oils. Their preferential viscosity and viscosity index improving effect makes possible a more extensive substitution of the traditional high molecular weight polymers. The feasibility of higher dosage level, of additives prepared according to the present invention starting from low molecular weight polyisobutylenes used so far for the preparation of ashless dispersants offers a more economic formulation of lubricants.

## Claims

1. An additive for use in an oil solution in lubricating oils of internal combustion engines, which contains imides and/or esters and/or ester amides of the reaction product of a poly-isobutylene of a number average molecular weight from 800 - 15 000, an unsaturated reactive dicarboxylic acid and/or its anhydride, preferably maleic anhydride, and another low molecular weight unsaturated comonomer,
wherein said reaction product contains on the average 1.6 - 6.0 dicarboxylic acid and/or its anhydride, preferably succinic anhydride groups per polyisobutylene chain,
in said reaction product the concentration of molecules containing more than one dicarboxylic acid and/or its anhydride, preferably succinic anhydride group, is more than 25%,
the widening of the molecular weight distribution of said reaction product is less than 70 percent, referred to the starting polyisobutylene,
and in said reaction product the polyisobutylene is grafted on or reacted with a dicarboxylic acid and/or its anhydride, preferably succinic anhydride containing copolymer formed from a low molecular weight unsaturated comonomer of a molecular weight less than 500, or from a mixture of such comonomers, and from an unsaturated reactive dicarboxylic acid and/or its anhydride, preferably maleic anhydride, using a molar ratio of 1.2 - 5.5 : 0.1 - 3.5 : 1 = dicarboxylic acid and/or its anhydride, preferably maleic anhydride : comonomer : polyisobutylene, and
said imides and/or esters and/or ester amides of said reaction product are obtained by reacting the dicarboxylic acid and/or its anhydride, preferably succinic anhydride groups of the copolymer linked to the polyisobutylene in a 0.7 - 5.5 ratio with at least bifunctional compounds containing one or more amine and/or hydroxyl groups.

2. The additive according to Claim 1, wherein said reaction product contains on the average 1.8 - 4.0 succinic anhydride groups per polyisobutylene chain.

3. The additive according to Claim 1, wherein the average number of molecules linked by the reaction of the carboxylic groups is between 2 and 100 in the components of various average molecular weight.

4. A process for preparing a detergent - dispersant additive, wherein a dicarboxylic acid and/or its anhydride, preferably maleic anhydride, and another low molecular weight comonomer with an olefinic double bond or their copolymers are grafted to a polyisobutylene of an average molecular weight from 800 - 15 000 by an addition reaction using the molar ratio 1.2 - 5.5 : 0.1 - 3.5 : 1 of dicarboxylic acid and/or its anhydride, preferably maleic anhydride : comonomer : polyisobutylene, where the solvent concentration providing homogeneous phase is 10 - 75 weight percent, preferably 35 - 60 weight percent with respect to the reaction mixture, carried out in the presence of 5 - 25 weight percent of a radical initiator and of 0.01 - 5 weight percent, referred to the dicarboxylic acid and/or its anhydride, preferably maleic anhydride, of a monomer incorporation ratio controlling component at 1 - 15x10² kPa pressure and preferably in nitrogen and/or hydrocarbon atmosphere, at 80 - 180° C, in 1 - 16 hours while the concentration of the dicarboxylic acid and/or its anhydride, preferably maleic anhydride, and the comonomer is kept below 5 weight percent, the obtained intermediate is stripped off from its solvent content and is diluted with refined base oil, if desired, and when it is necessary it is clarified and filtered in the presence of a filtration aid, the intermediate is reacted with at least bifunctional compounds containing one or more amine and/or hydroxyl groups, while the ratio of the compounds carrying the dicarboxylic acid and/or its anhydride, preferably succinic anhydride groups, and the amine and/or hydroxyl groups is 0.7 - 5.5, wherein the reaction is carried out, at 0.05 - 6x10² kPa pressure, at 120 - 235° C, in 2 - 15 hours and optionally in the presence of a catalyst in 0.1 - 2 weight percent, referred to the reaction mixture, and the product, if desired, is modified in a usual way, diluted and filtered.

5. The process according to Claim 4, wherein the reaction between the polyisobutylene, maleic anhydride and the comonomer is carried out in a solvent or in a mixture of solvents having hydrocarbon components of a boiling point less than 250° C in a concentration of at least 3 weight percent.

6. The process according to Claim 4, wherein the modification is carried out with compounds containing boron, sulfur, copper and/or molybdenum and/or polyalkenyl succinic anhydride or ester amide.

## Patentansprüche

1. Additiv zur Verwendung in einer Öllösung in Schmierölen für Verbrennungsmotoren, das Imide und/oder Ester und/oder Esteramide des Reaktionsproduktes eines Polyisobutylens mit einem zahlenmäßigen Durchschnittsmolekulargewicht von 800 bis 15.000 mit einer ungesättigten reaktionsfähigen Dicarbonsäure und/oder ihrem Anhydrid, vorzugsweise Maleinsäureanhydrid, und einem anderen niedermolekularen ungesättigten Comonomer,
wobei das Reaktionsprodukt durchschnittlich 1,6 bis 6,0 Gruppen einer Dicarbonsäure und/oder ihres Anhydrids, vorzugsweise Bernsteinsäureanhydridgruppen, pro Polyisobutylenkette enthält,
die Konzentration der mehr als eine Gruppe einer Dicarbonsäure und/oder ihres Anhydrids, vorzugsweise des Bernsteinsäureanhydrids, enthaltenden Moleküle über 25 % liegt,
die Erweiterung der Molekulargewichtsverteilung des Reaktionsproduktes, bezogen auf das Ausgangspolyisobutylen, weniger als 70 % beträgt und
im Reaktionsprodukt das Polyisobutylen auf das eine Dicarbonsäure und/oder ihr Anhydrid, vorzugsweise Bernsteinsäureanhydrid, enthaltendes Copolymer, das aus einem niedermolekularen gesättigten Comonomer mit einem Molekulargewicht von unter 500 oder aus einem Gemisch derartiger Comonomeren und aus einer ungesättigten reaktionsfähigen Dicarbonsäure und/oder ihrem Anhydrid, vorzugsweise Maleinsäureanhydrid, bei einem Molarverhältnis Dicarbonsäure und/oder ihr Anhydrid, vorzugsweise Maleinsäureanhydrid, : Comonomer : Polyisobutylen = 1,2 bis 5,5 : 0,1 bis 3,5 : 1 gebildet ist, aufgepfropft oder mit ihm umgesetzt ist, und
die Imide und/oder Ester und/oder Esterimide des Reaktionsprodukts durch Umsetzung der Gruppen der Dicarbonsäure und/oder ihres Anhydrids, vorzugsweise des Bernsteinsäureanhydrids, des mit dem Polyisobutylen in einem Verhältnis von 0,7 bis 5,5 verknüpften Copolymers mit wenigstens bifunktionellen, eine oder mehrere Amin- und/oder Hydroxylgruppen enthaltenden Verbindungen erhalten werden.

2. Additiv nach Anspruch 1, bei dem das Reaktionsprodukt durchschnittlich 1,8 bis 4,0 Bernsteinsäureanhydridgruppen pro Polyisobutylenkette enthält.

3. Additiv nach Anspruch 1, bei dem die durchschnittliche Zahl der durch die Umsetzung der Carboxylgruppen verknüpften Moleküle in den Ketten von unterschiedlichem durchschnittlichen Molekulargewicht 2 bis 100 beträgt.

4. Verfahren zur Herstellung eines als Detergens und Dispergator fungierenden Additivs, bei dem eine Dicarbonsäure und/ oder ihr Anhydrid, vorzugsweise Maleinsäureanhydrid, und ein anderes niedermolekulares Comonomer mit einer olefinischen Doppelbindung oder deren Copolymere auf ein Polyisobutylen mit einem durschschnittlichen Molekulargewicht von 800 bis 15.000 durch eine Additionsreaktion bei einem Molarverhältnis Dicarbonsäure und/oder ihr Anhydrid, vorzugsweise Maleinsäureanhydrid, : Comonomer : Polyisobutylen = 1,2 bis 5,5 : 0,1 bis 3,5 : 1 aufgepfropft werden, wobei die die homogene Phase liefernde Lösungsmittelkonzentration im Hinblick auf das Reaktionsgemisch 10 bis 75 und vorzugsweise 35 bis 60 Gew.-% beträgt und die Reaktion in Anwesenheit von 5 bis 25 Gew.-% eines Radikalinitiators und von 0,01 bis 5 Gew.-%, bezogen auf die Dicarbonsäure und/oder ihr Anhydrid, vorzugsweise Maleinsäureanhydrid, einer die Monomeraufnahme steuernden Komponente bei einem Druck von 1 bis 15x10² kPa und vorzugsweise in einer Stickstoff und/oder Kohlenwasserstoffatmosphäre bei 80 bis 180°C während 1 bis 16 Stunden durchgeführt wird, wobei die Konzentration der Dicarbonsäure und/oder ihres Anhydrids, vorzugsweise Maleinsäureanhydrids, und des Comonomers unter 5 Gew.-% gehalten wird, das erhaltene intermediäre Produkt vom Lösungsmittel abdestilliert und gegebenenfalls mit raffiniertem Basisöl verdünnt sowie gegebenenfalls geklärt und in Anwesenheit eines Filterhilfsmittels filtriert wird und danach mit wenigstens bifunktionellen, eine oder mehrere Amin- und/oder Hydroxylgruppen enthaltenden Verbindungen umgesetzt wird, wobei das Verhältnis der Gruppen der Dicarbonsäure und/oder ihres Anhydrids, vorzugsweise des Bernsteinsäureanhydrids, zu den Amin- und/oder Hydroxylgruppen 0,7 bis 5,5 beträgt, die Reaktion bei einem Druck von 0,05 bis 6x10² kPa bei 120 bis 235°C während 2 bis 15 Stunden und gegebenenfalls in Anwesenheit von 0,1 bis 2 Gew.-% eines Katalysators, bezogen auf das Reaktionsgemisch, durchgeführt wird und das Produkt, wenn erwünscht, auf die übliche Art und Weise modifiziert, verdünnt und filtriert wird.

5. Verfahren nach Anspruch 4, bei dem die Reaktion zwischen Polyisobutylen, Maleinsäureanhydrid und dem Comonomer in einem Lösungsmittel oder einem Lösungsmittelgemisch mit Kohlenwasserstoffkomponenten mit einem Siedepunkt von unter 250°C bei einer Konzentration von wenigstens 3 Gew.-% durchgeführt wird.

6. Verfahren nach Anspruch 4, bei dem die Modifizierung mit Bor, Schwefel, Kupfer und/oder Molybdän enthaltenden Verbindungen und/oder mit Polyalkenylbernsteinsäureanhydrid oder - esteramid durchgeführt wird.

## Revendications

1. Additif pour utilisation dans une solution huileuse dans des huiles lubrifiantes pour moteurs à combustion interne, qui contient des imides et/ou des esters et/ou des esters amides du produit de la réaction d'un poly-isobutylène d'un poids moléculaire moyen numérique de 800 à 15.000, d'un acide dicarboxylique réactif insaturé et/ou de son anhydride, de préférence l'anhydride maléique, et d'un autre comonomère insaturé de faible poids moléculaire,
dans lequel ledit produit de la réaction contient en moyenne 1,6 à 6,0 acides dicarboxyliques et/ou son anhydride, de préférence des groupes anhydride succinique, par chaîne de poly-isobutylène,
dans ledit produit de la réaction la concentration des molécules contenant plus d'un acide dicarboxylique et/ou son anhydride, de préférence le groupe anhydride succinique, est supérieur à 25%,
l'élargissement de la distribution des poids moléculaires dudit produit de la réaction est inférieur à 70 pour cent, par rapport au poly-isobutylène de départ,
et dans ledit produit de la réaction le poly-isobutylène est greffé sur ou mis à réagir avec un acide dicarboxylique et/ou son anhydride, de préférence l'anhydride succinique, contenant le copolymère formé à partir d'un comonomère insaturé de faible poids moléculaire, d'un poids moléculaire inférieur à 500, ou à partir d'un mélange de tels comonomères, et à partir d'un acide dicarboxylique réactif insaturé et/ou de son anhydride, de préférence l'anhydride maléique, en utilisant un rapport molaire de 1,2-5,5 :0,1-3,5 :1 = acide dicarboxylique et/ou son anhydride, de préférence l'anhydride maléique:comonomère:poly-isobutylène, et
lesdits imides et/ou esters et/ou esters amides dudit produit de la réaction sont obtenus en faisant réagir les groupes acide dicarboxylique et/ou son anhydride, de préférence l'anhydride succinique du copolymère lié au poly-isobutylène dans un rapport de 0,7-5,5 avec des composés au moins bifonctionnels contenant un ou plusieurs groupes amines et/ou hydroxyles.

2. Additif selon la revendication 1, dans lequel ledit produit de la réaction contient en moyenne 1,8 à 4,0 groupes anhydride succinique par chaîne de poly-isobutylène.

3. Additif selon la revendication 1, dans lequel le nombre moyen de molécules liées par la réaction des groupes carboxyliques est compris entre 2 et 100 dans les constituants de divers poids moléculaires moyens.

4. Procédé de préparation d'un additif détergent-dispersant, dans lequel un acide dicarboxylique et/ou son anhydride, de préférence l'anhydride maléique, et un autre comonomère de faible poids moléculaire comportant une double liaison oléfinique ou leurs copolymères sont greffés à un poly-isobutylène d'un poids moléculaire moyen de 800 à 15.000 par une réaction d'addition en utilisant un rapport molaire de 1,2-5,5 :0,1-3,5 :1 de l'acide dicarboxylique et/ou de son anhydride, de préférence l'anhydride maléique:comonomère:poly-isobutylène, dans lequel la concentration du solvant donnant la phase homogène est de 10 à 75 pour cent en poids, de préférence de 35 à 60 pour cent en poids par rapport au mélange réactionnel, en présence de 5 à 25 pour cent en poids d'un initiateur de la polymérisation radicalaire et de 0,01 à 5 pour cent en poids, par rapport à l'acide dicarboxylique et/ou son anhydride, de préférence l'anhydride maléique, d'un constituant de contrôle du rapport d'incorporation du monomère, sous une pression de 1 - 15 x 10² kPa et de préférence dans une atmosphère d'azote et/ou d'hydrocarbure, à 80-180°C, en 1 à 16 heures, pendant que la concentration de l'acide dicarboxylique et/ou de son anhydride, de préférence l'anhydride maléique, et du comonomère est maintenue en-dessous de 5 pour cent en poids, l'intermédiaire obtenu est débarrassé de sa teneur en solvant et est dilué avec une huile de base raffinée, si on le désire, et, si nécessaire, il est clarifié et filtré en présence d'un adjuvant de filtration, l'intermédiaire est mis en réaction avec des composés au moins bifonctionnels contenant un ou plusieurs groupes amines et/ou hydroxyles, pendant que le rapport des composés portant les groupes acide dicarboxylique et/ou son anhydride, de préférence l'anhydride succinique, et les groupes amines et/ou hydroxyles est de 0,7 à 5,5, dans lequel la réaction est effectuée sous une pression de 0,05 à 6 x 10² kPa, à une température de 120 à 235°C, en 2 à 15 heures et facultativement en présence d'un catalyseur à 0,1 à 2 pour cent en poids, par rapport au mélange réactionnel, et le produit, si on le désire, est modifié d'une façon habituelle, dilué et filtré.

5. Procédé selon la revendication 4, dans lequel la réaction entre le poly-isobutylène, l'anhydride maléique et le comonomère est effectuée dans un solvant ou dans un mélange de solvants ayant des constituants hydrocarbonés dont le point d'ébullition est inférieur à 250°C, à une concentration d'au moins 3 pour cent en poids.

6. Procédé selon la revendication 4, dans lequel la modification est réalisée avec des composés contenant du bore, du soufre, du cuivre et/ou du molybdène et/ou un anhydride succinique ou un ester amide de polyalkényle.
